

## UNITED STATES PATENT OFFICE

2,155,621

## RUBBER PROCESS AND PRODUCT

Thomas Lewis Shepherd, London, England

No Drawing. Application April 1, 1936, Serial  
No. 72,219. In Great Britain April 4, 1935

9 Claims. (Cl. 18—54)

This invention relates to rubber processes and products in which rubber is manufactured in thread, filament or tape form.

Rubber may be manufactured in such form by extruding latex with or without other ingredients such as vulcanisers, accelerators, reinforcing fillers, anti-oxidants and stabilisers.

In my U. S. applications Nos. 34,855 and 40,859 I describe processes in which there is mixed with the latex or latex mixture for extrusion purposes various setting agents, such as glue, gelatine and similar proteins, casein albumen or the like, natural and synthetic resins and gums which are water or alkali soluble, cuprammonium, cellulose ethers which are water or alkali soluble, e. g. methyl cellulose and substances, inorganic or organic, which dissolve in water or dilute alkalies to give solutions which are miscible with latex. When the latex mixture is extruded or otherwise formed into thread by coagulating the rubber, and dried, a set thread is produced, which may be woven or otherwise manipulated without the difficulties associated with extensible threads.

In my U. S. applications Nos. 11,720, 15,340, 66,308, and 66,309 processes are described in which rubber thread is provided after coagulation with a soluble or insoluble coating such as glue, gelatine, suitable cellulose derivatives, starch, wax, resin or the like, varnish, such as gum damar or copal, solutions of rubber or latex. By this means thread with no, or only a limited stretch, is produced, which may be incorporated in fabrics without the difficulties associated with the manipulation of extensible threads, and this thread may be rendered extensible in the case of the soluble coatings by dissolving the latter out.

The object of the invention is to improve or modify the threads or the processes described in the abovementioned specifications or applications, and in this way to produce a thread with improved properties more particularly from the point of view, among other things, of strength and of the property of being non-hygroscopic.

I have discovered that a thread which has been formed from latex and a setting agent may be greatly strengthened by providing it with a coating, and, at the same time, the coating is better able to attach itself to the thread when this is formed of rubber with a setting agent. I may or may not dissolve out the coating and setting agent and in a case when I do not, but, on the contrary, render the coating, for instance, gelatine insoluble by means of formaldehyde,

alum, potassium dichromate or the like, a thread will be produced which will be non-extensible and non-hygroscopic and suitable for incorporating in fabrics and if made with, at most, half the contents rubber and compounding materials is very suitable for imitation horsehair. I have found glue and gelatine to be very suitable setting and coating agents respectively.

The invention consists in a method for making thread which consists in coagulating a mixture of latex and setting agent and then applying a coating.

The invention also consists in a method as above, in which the setting agent is glue and the coating is gelatine.

The invention also consists in either of the methods as above, in which a flexiser, for example glycerine, is incorporated with the coating.

The invention also consists in any of the methods as above, in which the thread is coated with cellulose acetate or the like whilst it is still tacky.

The invention also consists in any of the methods as above, in which the thread is dyed at the same time as the setting agent and coating agent are removed.

The invention also consists in a method as in the preceding paragraph in which the thread is vulcanised at the same time as it is dyed.

The invention also consists in any of the methods as above, in which the setting agent and the coating are removed, leaving a rubber thread, which may or may not have a small proportion of setting agent left therein.

The invention also consists in any of the methods as above, in which dyestuff is mixed with the mixture of setting agent and latex.

The invention also consists in any of the methods as above, in which dyestuff is mixed with the coagulating agent.

The invention also consists in the method of the first statement of invention, in which the coating is rendered insoluble.

The invention also consists in a modification of any of the processes as above, in which the setting agent instead of being mixed with the latex is mixed with a coagulant for the latex.

The invention also consists in methods substantially as hereinafter described.

The invention also consists in thread when made by any of the methods as above.

The invention also consists in thread containing less than half rubber and compounding materials for rubber, the remainder being setting agent and coating for example 45 per cent.

or, at most, 45 per cent. rubber contents and compounding materials and 55 per cent. or, at least, 55 per cent. glue and gelatine.

The invention also consists in thread substantially as hereinafter described.

In carrying the invention into effect in one method by way of example, a mixture is prepared as follows:—

|    |                              |      |
|----|------------------------------|------|
| 10 | Revertex                     | 130  |
| 10 | Sulphur                      | 2.25 |
|    | Zinc oxide                   | 3.00 |
|    | Accelerator                  | 0.75 |
|    | Agerite white                | 0.50 |
| 15 | 10 per cent. casein solution | 5.00 |

15 This mix is warmed slightly and to it is added— whilst stirring is effected—50 per cent. glue solution in such a quantity as will correspond with 15 parts of dry glue to 85 of dry rubber. Such 20 a composition is extruded warm or even hot into a coagulation bath comprising a warm or hot solution of the following formula:—

|    |             |    |
|----|-------------|----|
| 15 | Acetone     | 85 |
| 25 | Acetic acid | 15 |

25 The coagulation bath solution need not of necessity be hot or warm but may also be cold and the extrusion or thread making point where the mix in thread form leaves the thread forming point is kept warm or hot or may be cold.

30 A thread prepared by extrusion and subsequent coagulation from a mix such as that above specified, is dried or dried and vulcanised. Further, to obtain an improved thread it may after coagulation be run into a bath or through a bath 35 of a liquid such as ethyl alcohol which will remove the majority of the water from the thread causing the precipitation of the glue. The thread after passing through or being left in the bath of alcohol or similar liquid is then dried and, 40 if desired, vulcanised. The thread obtained using the second bath of alcohol is more limited in stretch than that obtained using heat to remove the water. For the drying of the thread after 45 the treatment with alcohol a tunnel heated to a low temperature may be employed or the thread may be passed from the alcohol bath through starch or chalk or any suitable powdering agent, collected and allowed to dry at room temperature.

50 The coating may then be applied in any suitable way as by painting, spraying or otherwise, or the thread may be passed through a bath of the desired liquid so that it picks it up in 55 transit.

55 The thread may also be treated by coating a vulcanised or unvulcanised thread under a desired degree of stretch for instance 20-25 per cent. with a suitable kind of soluble adhesive. 60 Such an adhesive coating which may be a quick drying one may consist of glue, gelatine (equal parts by weight in water), a solution of a cellulose derivative, starch, molten wax, resin or the like, or a suitable varnish such as gum damar or copal. It may be applied by coating, spraying or otherwise, before the process of weaving. The coating will be applied and allowed to dry to such a degree as will impart to the thread a rigid or semi-rigid set so that 65 the resulting thread will not possess the characteristic of stretch, and is deprived of its elasticity or resilience as before.

70 As stated above, the adhesive used may be of such a character that it will quickly dry, but if

necessary the drying can be accelerated by artificial drying means of any kind.

The thread may be coated by suitable means (any known means) with a coating or skin of a gelatine solution, the strength of which may vary to a very great extent, say from 10 parts by weight of gelatine in 90 parts of fluid (water) up to 75 parts of gelatine by weight and 25 parts of fluid (water) to which may be added according to requirements certain quantities of flexiser, 10 more especially glycerine, varying from 3 per cent. (by weight) of the gelatine-water total up to 25 per cent. (by weight) of the gelatine-water total.

15 This gelatine coating may be dried in heat or in the ordinary atmosphere; it may, whilst leaving the warm or hot gelatine bath or shortly thereafter, be run through a fine powder, such as talcum powder, French chalk or flour or the like, so as to render it non-tacky, making it 20 possible to wind it.

The thread can, if desired, be left partially soluble, leaving, after dissolving most of the glue and gelatine, a rubber thread structure capable after incorporation into fabrics by means of 25 weaving, knitting or lacing and the like, of imparting to such fabrics a certain amount of elasticity.

It is to be understood that the threads ready for weaving may comprise either the uncoated 30 or uncovered rubber itself, or may comprise those with a winding thereon of silk, cotton, or other fibrous material.

As regards dyeing, thin threads up to 8000 yards to the pound dye right through fairly 35 easily in the cold, but thicker ones will not get dyed right into the core unless prolonged boiling in dyestuff is given of at least half an hour to one hour.

This is when this thread is still in the unvulcanised condition; when vulcanised, the thread must be dyed by means of a cold process 40 when there is a risk of over vulcanising the thread in the boiling process.

Practically the whole range of known dyestuffs 45 may be used.

As regards vulcanisation, in the normal procedure a boiling out of the setting agent will happen simultaneously with dyeing i. e., after the "set" and coated thread has been incorporated into fabric, i. e., in the grey cloth, this grey cloth is then dyed by boiling, causing the thread to be "de-set", to become flexible and to become vulcanised at the same time.

The vulcanisation takes place chiefly in the 55 dyeing-boiling process when the yarn is already in the piece, but in many instances I also vulcanise the thread after or before the gelatine coating has been applied so that the yarn, ready for weaving or knitting, is already vulcanised 60 or semi-vulcanised so that the subsequent boiling in the piece will either be short and of not sufficient duration to influence vulcanisation or to be so much as to complete the partial vulcanisation already given to the thread before its 65 incorporation in the fabric.

Instead of being extruded the thread may be formed by a disc method for example as in my U. S. applications Nos. 21,264 and 21,265, and in the case of extrusion coagulant may be extruded into latex, and/or the setting agent may be mixed with the coagulant as described in my U. S. application No. 40,859.

70 In a variation, the thread, when coming from the thread making machine and therefore in a 75

wet condition and tacky, may be coated with a solution of cellulose acetate or similar material, so as to coat the tacky thread with a very thin film of non-tacky material, whereby the thread 5 on arrival at the end of the heating and drying apparatus is absolutely non-tacky and can therefore be wound as required at once without stretch if so desired either direct on to a weaving pirn or in the form of a cheese, bobbin or the like.

10 The application of the cellulosic or like coating renders the thread absolutely non-tacky and it also prevents the thread from being rapidly affected by atmospheric moisture.

Various methods may be adopted for applying 15 such film, for example:

(a) The thread may be run into a normal coagulant, then passed through a dilute bath of cellulose acetate in acetone (about 5 per cent. strength) and then through a bath of water;

20 (b) The thread may be run into a bath containing acetic acid, acetone and the acetate, dispensing with water and allowing the heat in the heating chamber to dry off the solvents, thus leaving the surface in a non-tacky condition;

25 (c) The thread however prepared may be run through a normal coagulant passed through the acetate solution and then dried by passing it through a drying chamber, or

(d) The thread may be run into the ordinary 30 coagulant to which has been added a small quantity of acetate in acetone and then passing the thread through water and then drying.

Other materials besides cellulose acetate may be used, for example, substances which can be 35 dissolved in a volatile solvent and which may be easily separated from such solvent by heat, chemical action or any of the known methods, and leaving a non-tacky film.

As examples there may be mentioned cellulose 40 nitrate, viscose (to be precipitated in dilute acids), cellulose ethers and cellulose esters.

The term "latex" includes aqueous dispersions of rubber, gutta-percha, balata or similar materials.

45 I claim:

1. A method of preparing rubber thread in a relatively inextensible form which comprises the steps of forming a thread from an aqueous dispersion of rubber containing a quantity of a 50 removable lyophilic colloid sufficient to reduce the extensibility of the thread, coagulating the thread, drying the coagulated thread, applying to such thread a soluble adhesive coating which will be inextensible when hardened, and hardening the 55 coating.

2. A method of preparing rubber thread in a relatively inextensible form which comprises the steps of forming a thread from an aqueous dispersion of rubber containing a quantity of glue, sufficient to reduce the extensibility of the thread, coagulating the thread, drying the coagulated thread, applying to such thread a coating of gelatine, and hardening the coating.

3. A method as claimed in claim 2 in which the

thread contains approximately 55% of glue and gelatine which are rendered insoluble.

4. A method of preparing rubber thread in a relatively inextensible form which comprises the steps of forming a thread from an aqueous dispersion of rubber containing a quantity of glue, sufficient to reduce the extensibility of the thread, coagulating the thread, drying the coagulated thread, applying to such thread a coating of gelatine containing a plasticiser and hardening the 10 coating.

5. A method of preparing rubber thread in a relatively inextensible form which comprises the steps of forming a thread from an aqueous dispersion of rubber containing a quantity of glue, 15 sufficient to reduce the extensibility of the thread, coagulating the thread, drying the coagulated thread, applying to such thread a coating of a solution of gelatine containing glycerine and hardening the coating.

20 6. A method of preparing rubber thread in a relatively inextensible form which comprises the steps of forming a thread from an aqueous dispersion of rubber containing a quantity of a removable lyophilic colloid sufficient to reduce the 25 extensibility of the thread, coagulating the thread, applying a coating of cellulosic solution to the freshly formed thread and drying the coated thread.

7. A method of preparing rubber thread in a 30 relatively inextensible form which comprises the steps of forming a thread from an aqueous dispersion of rubber containing a quantity of a removable lyophilic colloid sufficient to reduce the extensibility of the thread, coagulating the 35 thread, applying a coating of cellulose acetate solution to the freshly formed thread and drying the coated thread.

8. A method of preparing a fabric in a relatively extensible form which comprises the steps 40 of forming a thread from an aqueous dispersion of rubber containing a quantity of a lyophilic colloid, sufficient to reduce the extensibility of the thread, coagulating the thread, drying the thread, applying a coating of soluble adhesive 45 which will be inextensible when hardened to the thread, hardening the coating, utilizing the thread to form a fabric and subsequently removing the lyophilic colloid and coating by means of a solvent therefor.

9. A method of preparing a fabric in a relatively extensible form which comprises the steps of forming a thread from an aqueous dispersion of rubber containing a quantity of lyophilic colloid sufficient to reduce the extensibility of 50 the thread, coagulating the thread, drying the coagulated thread, applying a coating of soluble adhesive which will be inextensible when hardened to the thread, hardening the coating, utilizing the thread to form a fabric and subsequently 55 simultaneously removing the lyophilic colloid and coating, and vulcanizing the thread by treatment of the fabric in a hot solvent for the lyophilic colloid and coating.

THOMAS LEWIS SHEPHERD.